

## UNITED STATES PATENT OFFICE

2,508,006

## CASTING MOLDS

Raymond E. Birch, Pittsburgh, Pa., assignor to  
 Harbison-Walker Refractories Company, Pittsburgh, Pa., a corporation of Pennsylvania

No Drawing. Application February 21, 1947.  
 Serial No. 730,189

4 Claims. (Cl. 22—188)

1

This invention relates to molds and mold parts of the sand, or non-permanent, type for the casting of metals and alloys, more particularly those cast at temperatures of at least about 1400° C.

Unless the contrary appears from the context, the word "sand" is used herein to refer not only to silica sand, crushed quartz and the like materials composed largely or substantially wholly of silica ( $\text{SiO}_2$ ), but also broadly includes other refractory materials that are used in subdivided form for the making of metal casting molds and mold parts. A variety of such other materials are known, examples being magnesite, zircon and olivine.

A major object of the invention is to provide refractory molds and mold parts, such as cores, for the making of metallic castings, that are easily prepared in accordance with standard practices, and which are characterized by undergoing dusting, or mechanical disruption, of the refractory sand adjacent the formed casting whereby stripping of the casting is facilitated and adherence of the refractory to the surface of the casting is minimized or eliminated.

A further object is to provide refractory compositions for making molds and mold parts, or for the surfacing of metal-contacting areas thereof, which are characterized by possessing the properties requisite for such uses and additionally of undergoing dusting in the regions adjacent the formed casting during and after cooling of the cast metal.

Still another object is to provide an improved method of casting metals and alloys, particularly those melting or castable above about 1400° C., which results in dusting of the mold material in contact with the cast metal during or after cooling whereby to insure easy stripping of the casting with minimized adherence of the mold material thereto.

Yet another object is to provide compositions, molds and a method in accordance with the foregoing objects that are applicable not only to sand type molds but also to the casting of metals and alloys in other ways including, by way of example, dental and the like investment castings.

Other objects will be recognized from the following specification.

Calcium orthosilicate, or dicalcium silicate ( $2\text{CaO} \cdot \text{SiO}_2$ ), is a highly refractory material capable of existing in three allotropic modifications, i. e., an alpha crystal form that is stable above about 1420° C., a beta form that is stable in the range from about 1420° to 675° C., and a gamma modification that is stable below about

2

675° C. As has been known for many years, the inversion from the beta to the gamma allotropic modification involves an increase in volume that apparently takes place instantaneously and which results in mechanical disintegration of the crystal grains, a phenomenon known to those familiar with it as dusting.

In the refractory art the presence of calcium orthosilicate in refractory materials has been considered undesirable because of the tendency to disruption of refractory shapes when they are cooled to or below the beta-gamma inversion temperature, and the presence of this mineral has been tolerated in refractories only when stabilized against that inversion by certain oxides such, for example, as  $\text{Cr}_2\text{O}_3$ ,  $\text{P}_2\text{O}_5$ ,  $\text{B}_2\text{O}_3$ ,  $\text{V}_2\text{O}_5$ , and  $\text{Mn}_2\text{O}_3$ .

Despite the prior beliefs that the dusting of calcium orthosilicate is undesirable and objectionable in refractories, I have found, and it is upon this that the invention is in large part predicated, that this phenomenon is advantageously utilized in the casting of metals in non-permanent, or sand, molds. More particularly, I have found that the stated objects of the invention are attained by having calcium orthosilicate in an unstabilized condition present in at least the metal-contacting surfaces of refractory molds whereby after the cast metal has cooled to or below the temperature at which the beta form inverts to the gamma form, the refractory material adjacent the casting will be disintegrated, or dusted. The significance of this self-powdering of the refractory material adjacent the casting is that it renders stripping of the castings from the molds easier, and the castings are freer from adherent refractory than is the case with molds of the same class used heretofore. Accordingly, the invention results not only in more rapid and easier stripping of castings from the molds than heretofore, but also, the previously necessary laborious and time-consuming operation of cleaning the castings to remove adherent refractory is reduced, or even eliminated.

The invention may be practiced in various ways. Thus, the metal-contacting surfaces, or mold cavities, of ordinary silica sand or other non-permanent types of molds made from refractory materials may be surfaced with material supplying unstabilized calcium orthosilicate in accordance with the invention. Or, the entire mold or mold parts, such as cores, may be made from refractory substances adapted to provide unstabilized calcium orthosilicate under the heat of the cast metal. In all such embodiments the

mold or the facing material may consist wholly of materials reactive to provide calcium orthosilicate, or it may be made up of refractory materials adapted to provide certain predetermined proportions of the unstabilized silicate.

Similarly, the unstabilized calcium orthosilicate may be provided in various ways, as will appear hereinafter.

In the preferred practice of the invention unstabilized calcium orthosilicate is formed by reaction in situ in the mold substance under the heat supplied by the cast metal. Thus, metal casting molds and parts thereof may be made from refractory material containing lime and silica in forms and in amounts such that unstabilized calcium orthosilicate will be formed when metal is cast in the mold and will undergo the beta-to-gamma inversion upon cooling the casting in the mold.

I now believe that with materials productive of calcium orthosilicate in the forms in which they would most commonly be used in molds react at a rate satisfactorily productive of effective amounts of the orthosilicate at temperatures over about 1300° or 1400° C., and that consequently, the invention is particularly applicable to those metals and metal alloys that are normally cast at such temperatures, such as ferrous alloys and the precious and the high melting metals and their alloys, or other metals or alloys that may be cast satisfactorily at such temperatures. Nevertheless, it is entirely possible for this orthosilicate to be formed at lower temperatures, and particularly in the case of materials in states conducive to enhanced activity such, for example, as slaked lime and silica in an active form, e. g., precipitated silica or silica gel. Accordingly, the invention is not restricted to cases where the metal is cast at or above 1300° or 1400° C. but is rather applicable wherever sufficient calcium orthosilicate can be supplied to effect the desired dusting.

Calcium orthosilicate is theoretically composed of 65 per cent of CaO and 35 per cent of SiO<sub>2</sub> and for the purposes of the invention the refractory material consists of or contains those constituents substantially in those proportions. However, as will appear, the proportions may be varied somewhat from that theoretical composition. It is important, and critical, however, that however supplied the limits indicated by the data given hereinafter be not extended substantially for if they are, other calcium silicates may be formed in amounts that interfere with or prevent the dusting action that is essential to the invention. This refers, of course, to the actual material productive of dusting, i. e., the calcium orthosilicate. For example, this may be due to particles of lime or of silica converted throughout to the orthosilicate. Equally, however, sufficient of the orthosilicate may be formed on the surfaces of granules, e. g., of quartz, to cause the desired dusting on cooling; in such a case it is the composition of the orthosilicate coating that is important, not the overall composition of the particle which may be very different.

In general, as little as 10 per cent by weight of unstabilized calcium orthosilicate suffices to effect adequate dusting of various refractory sands, as that word is used herein, but larger amounts are generally preferable, and the refractory may even be converted wholly to the orthosilicate, particularly when applied merely as a mold facing.

The most obvious example of a suitable composition for practicing the invention is to mix

lime (CaO) and silica (SiO<sub>2</sub>) in proportions productive of calcium orthosilicate. For most purposes, however, it is preferable to adjust the composition of refractory materials adapted to the production of sand-type molds by the addition of one or more materials that provide unstabilized calcium orthosilicate in the refractory and which exert no specific influence on the molds or the castings, as by blending refractory materials containing lime and silica, naturally or added, so that they are present in proportions and amounts productive of enough calcium orthosilicate to cause the desired dusting.

The latter procedure can be illustrated by reference to the blending of two dead burned magnesites, designated A and B, whose analyses are given in the following table. In the blending of those magnesites to yield unstabilized calcium orthosilicate it is advisable, as indicated, to aim at a mixture containing lime and silica in the ratio of 65:35 by weight. By calculation this requires 30 per cent of magnesite A and 70 per cent of magnesite B, and the resultant blend will have the analysis indicated in the table as composition C. This gives a total of lime-plus-silica of 18.9 per cent, which is the maximum amount of dicalcium silicate that can form in the blend.

| 30 | Analysis                                | A                   | B                             | C                |
|----|-----------------------------------------|---------------------|-------------------------------|------------------|
|    |                                         | High Lime Magnesite | Standard Washington Magnesite |                  |
| 35 | MgO.....                                | Percent<br>62.90    | Percent<br>82.81              | Percent<br>77.00 |
|    | R <sub>2</sub> O <sub>3</sub> .....     | 3.69                | 4.30                          | 4.11             |
|    | CaO.....                                | 28.51               | 5.44                          | 12.27            |
|    | SiO <sub>2</sub> .....                  | 4.90                | 7.35                          | 6.62             |
|    | Ratio of CaO/SiO <sub>2</sub> (approx.) | 85/15               | 43/57                         | 65/35            |

The term "R<sub>2</sub>O<sub>3</sub>" in the foregoing table is used in conformity with common practice in the ceramic art to refer to the total content of sesquioxides, in this case alumina and iron oxide reported as Fe<sub>2</sub>O<sub>3</sub>. The term is used in this way in, for example, Patents Nos. 2,278,454 and 2,292,644, as well as at pages 50 and 51 of Ceramic Tests and Calculations by A. I. Andrews (1928).

Experience has shown that with dead burned magnesites the practical range in CaO : SiO<sub>2</sub> ratio is from 68:32 to 60:40, but little more. As will appear, the range may be somewhat wider with other refractories.

In the practice of the invention molds and mold parts, such as cores, are made in the manner customary in the trade, there being nothing in the nature of the compositions used that requires any change from existing sand mold practices. Thus, no change is necessary ordinarily in the grain size or range of grain sizes of the refractories, or sands, and the standard bonding agents may be used including such well known bonds as bentonite, clay, eyrite, cement, lignin extracts, cellulose lye, molasses, oils, resins, etc. Care should be taken, however, in selecting the refractory materials to avoid those containing stabilizing agents for the calcium orthosilicate, such as those named above, although small amounts of such agents will not be detrimental provided they are not present in amounts that effect stabilization of the orthosilicate against the beta-gamma inversion upon cooling. The mold units may be baked or dried in the usual manner.

After the molds have been prepared the metal is cast in them in the usual manner, and the

castings are allowed to cool at least to the temperature at which the dusting occurs, after which they may be stripped readily from the molds and, as indicated above, there will usually be no substantial adherence of the refractory to the castings such as is encountered in the use of ordinary sand molds. Even if some of the refractory becomes attached to the surface of the casting, the bond will be only temporary because on cooling, or on standing for a short interval, the calcium orthosilicate in the fused material will recrystallize and undergo dusting, and thereby substantially free the casting from adherent refractory.

The compositions used in the practice of the invention are capable of re-use because normally the portion of the mold that dusts will represent only a thin reacted layer next to the metal. If judged necessary to remove the dusted material, this can be done readily by allowing the powder to fall away before crushing the mold for re-use, or by screening out the dust. However, the dusted powder will do no harm except that build-up in successive batches arising from re-use of the molds will in time reduce the permeability of the mold to an extent that may be objectionable. Naturally, it is good practice when re-using these refractory materials to mix some new batch with the old before re-using it.

Although, as indicated above, the entire mold may be made from compositions in accordance with the invention, it is entirely feasible to use such compositions only for facing the mold cavity or other metal-contacting surfaces, such as the surfaces of cores, which will be in direct contact with the casting. Generally speaking, such facings may be about  $\frac{1}{4}$  to  $\frac{3}{4}$  inch thick. This facing layer may extend over the entire mold cavity or only where the greatest trouble due to adherence of sand to castings is anticipated. In this way cheaper sands or other refractory materials may then be used for back-up, and in general for those parts of the mold that do not affect the surface of the casting at vital points. The use of compositions yielding calcium orthosilicate, whether to constitute the entire mold or only a facing as just described, does not interfere in any way with the well-known practices of using thin wash or brush coatings of graphite, calcined clay, silica flour, olivine dust, or other materials commonly applied to finished mold surfaces.

As a further example of compositions in accordance with the invention, reference may be made to the blending of Portland cement and dead burned magnesite, the former of which typically has a  $\text{CaO:SiO}_2$  ratio higher than that of dicalcium silicate, and the latter of which has a lower ratio than the desired resultant. In one series of tests there were used cement and dead burned magnesite of the following composition:

|                                         | Dead-Burned<br>Magnesite | High Early<br>Strength<br>Portland<br>Cement |
|-----------------------------------------|--------------------------|----------------------------------------------|
|                                         | Per Cent                 | Per Cent                                     |
| $\text{SiO}_2$ .....                    | 4.9                      | 20.6                                         |
| $\text{Al}_2\text{O}_3$ .....           | 2.0                      | 6.0                                          |
| $\text{Fe}_2\text{O}_3$ .....           | 3.5                      | 2.7                                          |
| $\text{CaO}$ .....                      | 2.4                      | 65.1                                         |
| $\text{MgO}$ .....                      | 86.5                     | 1.6                                          |
| $\text{SO}_3$ .....                     |                          | 2.4                                          |
| Total.....                              | 99.3                     | 98.4                                         |
| Ratio $\text{CaO:SiO}_2$ (approx.)..... | 33/67                    | 76/24                                        |

Using these two materials ground to pass 65 mesh, 3 mixes were made up as follows, and in

each instance they were molded into cylinders after adding 5 per cent of water and 2 per cent of lignin liquor to give a temporary bond:

| Mix                                     | Mix #1 | Mix #2 | Mix #3 |
|-----------------------------------------|--------|--------|--------|
| Magnesite..... per cent                 | 80     | 75     | 70     |
| Cement..... do.....                     | 20     | 25     | 30     |
| Calc. $\text{CaO:SiO}_2$ (approx.)..... | 65/35  | 67/33  | 69/31  |

10 The molded cylinders were heated to  $1400^{\circ}\text{C}$ . to cause the formation of calcium orthosilicate, as would occur in a casting operation. The test pieces were then cooled, and upon inspection it was found that mix #1 was cracked, and that it completely powdered after 24 hours. Mix #2 powdered completely without delay, while mix #3 did not show dusting for several days. It follows that in this instance the ratio



was better, from the standpoint of prompt dusting, than the theoretical 65:35 ratio, and that the practical dusting range does not extend to a ratio of 69:31. These tests show also that the dusting inversion does not invariably occur at the normal inversion temperature of  $675^{\circ}\text{C}$ ., but that a metastable state may exist which will delay inversion and dusting for some hours, in view of which castings made in such molds may clean more readily if there is some delay in stripping them from the molds. The reason why dusting was more effective with these mixes at a  $\text{CaO:SiO}_2$  ratio of 67:33 than at the 65:35 ratio is probably to be found in the influence of the minor constituents of the mix, or it may be due to the magnesia or alumina.

20 In some instances there would be no objection to a strong set such as may be obtained by Portland cement, and in those cases it may be advantageous to use enough water not only to cause full setting of the mix, but enough actually to make molds by casting the mix around the pattern. On the other hand, in other instances the hydraulic action of the cement may give a stronger set than desired. This, however, is a familiar problem in the foundry that is taken care of variously, as by the known use of a limited amount of water to prevent attainment of full set, or by the use of oils instead of water, which is particularly feasible when the compositions are used only for facing the mold.

25 Although the invention has been described in detail with reference to the provision of the desired unstabilized calcium orthosilicate by reaction under the heat of the castings, and although it is preferred to practice the invention in that manner, equivalent results within the scope of my invention may be achieved simply by providing in the mold or the mold facing beta calcium orthosilicate held temporarily in an unstabilized metastable form whereby the heat supplied by the cast metal will cause the inversion to the gamma form to occur, with dusting, upon cooling the casting and mold assembly. Thus, dead burned magnesites can be produced with about 20 to 30 per cent of unstabilized dicalcium silicate held in the beta form almost permanently at normal room temperatures if the product is quickly cooled, or chilled, upon emergence from the rotary kiln in which it is produced. The beta form will apparently continue indefinitely in such a product unless and until the magnesite grain is again heated and then slowly cooled. Such a material containing the beta modification held

in a metastable condition as the result of an initial quick cooling can, of course, be used for the production of molds and the making of castings in accordance with my invention because, to repeat, the heat supplied by the molten metal and the slow cooling of the mold and its contained casting will cause inversion of the calcium silicate to the stable gamma form with dusting of that part of the molding composition adjoining the casting.

It is to be understood that any refractory base material, or combination of such materials may be used for making the molds that supply the properties requisite for such purposes together with the provision of enough calcium orthosilicate to effect dusting. Suitable ingredients particularly for supplying the unstabilized calcium orthosilicate are dolomite, limestone, calcium and magnesium silicates, wollastonite, pyroxene, amphibole, silica sand, sandstone, quartzite, serpentine, olivine and slags. Where raw materials exhibiting high shrinkage are used, such as dolomite and limestone, primary calcination is ordinarily desirable.

A readily dustable mix has been made, for example, by the blending of 56.1 per cent of Mg-Fe olivine sand or dunite from North Carolina with 43.9 per cent of hydrated lime to give a mix with a CaO : SiO<sub>2</sub> ratio of 65:35. Similarly good results were obtained using dolomitic lime in place of high calcium lime. Work with mixtures of dolomite and olivine gave the free dusting desired with all CaO : SiO<sub>2</sub> ranges from 58:42 to 69:31. The olivine used analyzed 39.6 per cent SiO<sub>2</sub>, 47.6 per cent MgO, 8.6 per cent FeO, and only a trace of CaO. Mixtures of potters flint and crude dolomite give dusting in the same range.

As an example of a three component mix in accordance with the invention, there may be used any combination of serpentine, dead burned magnesite, and a calcareous ingredient such as cement or lime provided the proportions are such as to effect the provision of calcium orthosilicate, suitably approximately 65 per cent CaO and 35 per cent SiO<sub>2</sub>. If the magnesite constitutes about 20 per cent, the mixes will be free from excessive shrinkage.

There may be used also as a mold material a mixture of silica sand, or a silicate, and a pre-fired calcium ferrite clinker.

Although the invention has been described thus far with particular references to sand-type molds, it is to be understood that the making of castings, such as dental castings, of the precious or the highly refractory metals in molds of investment compositions is not excluded in the practice of this invention. It is believed by some that in the making of dental castings, gypsum-Portland cement investments are objectionable because of the sulfur contained in the gypsum. An advan-

tage of the present invention for such purposes is that the presence of CaO appears to prevent sulfur damage of the castings. The compositions used in the practice of the invention are applicable also with advantage in the fusion casting of refractories, particularly those of basic compositions.

According to the provisions of the patent statutes, I have explained the principle and mode of practicing my invention, and I have described what I now consider to represent its best embodiment. However, I desire to have it understood that, within the scope of the appended claims, the invention may be practiced otherwise than as specifically described.

I claim:

1. A refractory mold or mold part for the casting of metal having at least the metal-contacting surface portion composed of refractory material containing, by chemical analysis, lime and silica substantially between the weight ratios 58CaO : 42SiO<sub>2</sub> and 69CaO : 31SiO<sub>2</sub> and reactive when heated by the cast metal to at least about 1300° C. to provide at least about 10 per cent of unstabilized calcium orthosilicate based on the weight of said material, said orthosilicate undergoing dusting at the surface of the casting after cooling it in the mold below the temperature at which the beta modification of said orthosilicate inverts to the gamma form.

2. A mold according to claim 1, said ratio being substantially 65CaO : 35SiO<sub>2</sub>.

3. A refractory mold or mold part according to claim 1, said refractory material comprising a mixture of dead burned magnesites.

4. A refractory mold or mold part for the casting of metal having at least the metal-contacting surface portion composed of dead burned magnesite containing about 20 to 30 per cent of unstabilized calcium orthosilicate in the beta modification and in a metastable state and which inverts to the gamma form and undergoes dusting at the surface of the casting after cooling of the casting in the mold below about 675° C.

RAYMOND E. BIRCH.

#### REFERENCES CITED

The following references are of record in the file of this patent:

#### UNITED STATES PATENTS

| Number    | Name    | Date          |
|-----------|---------|---------------|
| 1,077,958 | Gleason | Nov. 4, 1913  |
| 1,303,097 | Menee   | May 6, 1919   |
| 2,220,703 | Bean    | Nov. 5, 1940  |
| 2,391,855 | Bean    | Dec. 25, 1945 |

#### OTHER REFERENCES

Audley: "Silica and the Silicates," pages 52-54.  
Johnson: "Materials of Construction," 5th edition, pages 302 and 303.